

1

2,828,262

## SOAP-SALT COMPLEX THICKENED GREASE COMPOSITIONS

Arnold J. Morway, Clark, N. J., assignor to Esso Research and Engineering Company, a corporation of Delaware

No Drawing. Application April 19, 1955  
Serial No. 502,519

7 Claims. (Cl. 252—33.6)

This invention relates to new and improved lubricating grease compositions. More particularly, the invention pertains to lubricating oil base stocks thickened to grease consistency with soap-salt complexes comprising a metal salt of low molecular weight carboxylic acids, a metal salt of an alkylene diamine tetra carboxylic acid, and a metal soap of high molecular weight carboxylic acids.

In brief compass, the present invention relates to compositions consisting of or containing complex compounds consisting of a metal salt of a low molecular weight carboxylic acid containing from about 1 to 3 carbon atoms per molecule, a metal salt of an ethylene diamine tetra aliphatic carboxylic acid containing 1 to 4 carbon atoms in the aliphatic acid group and a metal soap of a high molecular weight carboxylic acid containing from about 12 to 30 carbon atoms per molecule. Grease compositions containing the complex compounds of the invention have been found to be suitable for lubricating services operating over a broad range of temperatures and under conditions of high unit load or boundary lubricating conditions.

The use of soap-salt complexes as grease thickeners is well known in the art. The complex compounds used heretofore consisted of combinations of metal soaps of high molecular weight carboxylic acids and metal salts of low molecular weight carboxylic acids. The commonly known grease-making, high molecular weight fatty acids, saturated or unsaturated, having from 12 to 22 carbon atoms have been employed in conjunction with such low molecular weight carboxylic acids, as acetic, propionic alkoxy propionic and the like to form the complex grease thickeners of the prior art.

In U. S. Patent No. 2,680,094, issued to Bartlett et al., the use of esters or metal salts of esters of ethylene bis-imino aliphatic carboxylic acids, i. e. ethylene diamine tetra aliphatic carboxylic acids, are disclosed as rust inhibiting lubricating oil additives. The preparation of the rust preventive additives of the Bartlett et al. patent involved esterifying the nitrogen-containing complex acids with aliphatic alcohols having between about 4 and 18 carbon atoms per molecule.

It has now been found that metal salts of alkylene diamine tetra aliphatic carboxylic acids having from 1 to 4 carbon atoms in the aliphatic carboxylic acid group can be utilized in conjunction with metal salts of low molecular weight carboxylic acids and metal soaps of high molecular weight carboxylic acids to prepare soap-salt complexes capable of thickening lubricating oils to grease consistency and imparting excellent load carrying characteristics to the final grease composition. By em-

2

ploying the alkylene diamine tetra carboxylic acids there is obtained a high combined metal content in the grease compositions with extremely high load carrying abilities without employing large amounts of salts and soaps. It has also been found that grease prepared in accordance with the invention will still retain adequate load carrying properties after they have been diluted or blended to make softer greases.

The low molecular weight carboxylic acids contemplated in this invention include saturated and unsaturated monocarboxylic acids having from about 1 to 3 carbon atoms per molecule, such as formic, acetic, propionic, lactic, acrylic and similar acids. Acetic acid is especially preferred and may be employed in the form of glacial acetic acid or concentrated aqueous solution containing from about 60 to 99.9 wt. percent, preferably about 80 wt. percent, of acetic acid. In general, the low molecular weight carboxylic acid employed should have a saponification value of above about 600, preferably about 900. Suitable high molecular weight carboxylic acids are those containing from about 12 to 30 carbon atoms, preferably from about 18 to 22 carbon atoms, per molecule. These acids may be derived from saturated or unsaturated naturally occurring or synthetic fatty material.

The fatty acids normally used in the manufacture of conventional grease thickeners, particularly the more saturated acids, are preferred. Examples of such acids include lauric, myristic, palmitic, stearic, mono-hydroxy stearic, di-hydroxy stearic, poly-hydroxy stearic, arachidic, hydrogenated fish oil, tallow acids, etc. However, unsaturated acids such as oleic, ricinoleic and similar acids may also be employed. The average saponification value of the high molecular weight monocarboxylic acids useful for the purposes of the present invention should not be more than about 300, preferably not more than about 220.

The nitrogen-containing complex acids, suitable for the purposes of this invention are the alkylene diamine tetra aliphatic carboxylic acids having the following approximate formula



wherein R is an alkyl group having from 1 to 4 carbon atoms. Ethylene bis-imino diacetic acid is commercially available from the Alrose Chemical Co. under the trade name "Sequestrene AA." The tetra- or trisodium salts are also commercially available under the trade name "Versene" from the Bersworth Chemical Co. Although ethylene diamine tetra acetic acid is preferred, the acids may be derived from other low molecular weight aliphatic carboxylic acids having from 1 to 4 carbon atoms per molecule.

The choice of metal component depends to a certain extent on the use of the soap-salt complexes of the invention. The alkaline earth metals such as calcium, barium, strontium and magnesium are particularly useful for many purposes of the invention. Calcium is especially preferred. These metals afford the greatest advantages when the soap-salt complexes are used as grease thickeners, since they result in the production of greases having outstanding load carrying characteristics even without the use of conventional extreme pressure agents.

The metal components of the salts and soaps may be any one or more of the metals set forth above. In most cases, however, the salts and soaps contain the same metal or combination of metals.

The soap-salt complexes of the invention may be utilized in combination with a wide variety of mineral as well as synthetic lubricating oils. Relatively large proportions of active metal may thus be introduced into the oils without solubility problems. Mineral base lubricating oils ranging in viscosity from about 50 to 2000 S. U. S. at 100° F., 35 to 100 S. U. S. at 210° F., are preferably employed as the liquid phase of the grease compositions of the invention. These naturally occurring mineral lubricating oils may be derived from any crude source, whether paraffinic or naphthenic in origin, which are refined by any of the well known refining techniques.

The invention is not limited, however, to the use of mineral base oils, since various synthetic oils may also be used as part or all of the liquid phase of the grease. Examples of operable synthetic oils include ether alcohols, such as those corresponding to the general formula



wherein R is an alkyl group, e. g. butyl, n is an integer from 1 to 5, and x is an integer greater than 1; esters of monobasic carboxylic acids, totaling 20 to 130 carbon atoms, such as those of C<sub>4</sub> to C<sub>18</sub> aliphatic acids with C<sub>4</sub> to C<sub>18</sub> aliphatic alcohols, the C<sub>4</sub> to C<sub>18</sub> radicals including the butyl, isobutyl, hexyl, octyl, iso-octyl, 2-ethyl hexyl, noyl, decyl, lauryl, stearyl and similar radicals; diesters of dibasic acids, such as adipic or sebacic acid with monohydric alcohols, such as hexyl, octyl, 2-ethyl hexyl or higher alcohols; esters of polyethylene glycols with C<sub>8</sub> to C<sub>18</sub> branched-chain carboxylic acids; complex esters of polybasic carboxylic acids, polyhydric alcohols, monobasic acids and/or monohydric alcohols, such as the well known glycol-centered or dibasic acid-centered complex esters; phosphoric acid esters of thioesters of aliphatic alcohols or mercaptans of up to about 18 carbon atoms; halocarbon oils, such as the polymers of chlorofluoroalkylenes like chlorotrifluoroethylene; organo-siloxanes; sulfite esters; organic carbonates; mercaptals; formals; etc.

In general, greases containing the thickeners of this invention are prepared by dispersing high molecular weight fatty acids and alkylene diamine tetra carboxylic acid with metal base in a portion or all of the lubricating oil to be used in the grease. The mixture is then heated to a temperature of about 80 to 130° F. with mixing. The low molecular weight carboxylic acid is then added. If only a portion of the lubricating oil was added initially, the remaining portion can be added at this point along with the low molecular weight carboxylic acid. Heating is continued to a temperature of about 400° to 550° F. The heating is then discontinued, and the grease batch cooled to a temperature of about 200 to 250° F. with agitation. At this temperature any of the conventional grease additives, e. g. oxidation inhibitors, such as phenyl alpha naphthylamine, can be added. The grease batch is then cooled to a temperature below about 180° F., and Gaulin homogenized.

The grease compositions of the invention can also be prepared by neutralizing all of the carboxylic acids employed in situ in the liquid menstruum to which the complex compound is to be applied in actual use.

The soap-salt complexes may also be prepared by separately preforming at least a portion of either the metal salt of the low molecular weight carboxylic acids, the metal salt of the ethylene diamine tetra carboxylic acids or the metal soap of the high molecular weight carboxylic acids. This method is particularly useful when different metals are employed as the metal constituents of the salts and soaps.

When the soap-salt complexes are prepared in a liquid dispersant or solvent, they may be isolated by solvent ex-

traction of the dispersing medium in a solvent in which the complex is insoluble. Suitable solvents include acetone, ether, hexane, etc.

As previously mentioned, the lubricating grease compositions of the invention can be diluted or blended with from about 10 to 70 wt. percent, preferably 25 to 50 wt. percent, of a mineral or synthetic lubricating oil to make softer greases having excellent load carrying characteristics.

In preparing the lubricating grease compositions of the invention about 50 to 97 wt. percent of lubricating oil and about 3 to 50 wt. percent of soap-salt complex are employed. The preferred grease compositions contain from about 5 to 30 wt. percent of the soap-salt complex containing from about 5 to 20 wt. percent of a low molecular weight carboxylic acid, from about 1 to 5 wt. percent of an ethylene diamine tetra carboxylic acid and from about 3 to 15 wt. percent of high molecular weight carboxylic acids. Thus, the complex itself is formed from 1 to 5 parts by weight of the ethylene diamine tetra carboxylic acid, 5 to 20 parts by weight of the low molecular weight carboxylic acid, and 3 to 15 parts by weight of the high molecular weight carboxylic acid. The amount of metal base employed will ordinarily be within the range of about 5 to 15 wt. percent, all of the above weight percentages being based on the total weight of the final grease compositions.

The invention will be more fully understood by reference to the following example, which illustrates various modifications of the invention:

#### EXAMPLE

To demonstrate the effect of employing a metal salt of ethylene diamine tetra aliphatic carboxylic acid in conjunction with a metal salt of a low molecular weight carboxylic acid and a metal soap of a high molecular weight carboxylic acid, a number of grease compositions, having the formulations and properties tabulated below, were prepared as follows:

#### Composition A

All of the mineral lubricating oil, hydrated lime and stearic acid were charged to a fire heated kettle and warmed to 135° F. while stirring. The acetic acid was added, and the mixture then heated to a temperature of about 500° F. At this temperature heating was discontinued, and the grease mixture cooled to about 250° F. with stirring. Phenyl alpha naphthylamine was then added. The resulting grease mixture was cooled to a temperature below about 180° F., and Gaulin homogenized at 6500 p. s. i.

#### Composition B

All of the mineral lubricating oil, hydrated lime, stearic acid and ethylene diamine tetra acetic acid were charged to a fire heated kettle and warmed to about 135° F. with stirring. The acetic acid was then added, and heating continued to a temperature of about 500° F. Heating was then discontinued, and the grease mixture cooled to about 250° F. with agitation. At this temperature phenyl alpha naphthylamine was added, the resulting grease mixture cooled to a temperature below about 180° F., and then Gaulin homogenized at 6500 p. s. i.

#### Composition C

This grease composition was prepared by blending about 75 wt. percent of Grease B with about 25 wt. percent of a mineral lubricating oil having a viscosity of 70 SUS at 210° F. at a temperature of about 200° F.

#### Composition D

This grease composition was prepared by blending about 75 wt. percent of Grease A with about 25 wt. percent of a mineral lubricating oil having a viscosity of 70 SUS at 210° F. at a temperature of about 200° F.

TABLE

| Grease Composition No.                                | A                            | B                | C                | D       |
|-------------------------------------------------------|------------------------------|------------------|------------------|---------|
| Formulation (Wt. percent):                            |                              |                  |                  |         |
| Glacial acetic acid                                   | 8.0                          | 12.0             | 9.0              | 6.00    |
| Stearic acid                                          | 4.0                          | 4.0              | 3.0              | 3.00    |
| Ethylene diamine tetra acetic acid                    |                              | 2.0              | 1.5              |         |
| Hydrated lime                                         | 6.0                          | 10.0             | 7.5              | 4.50    |
| Phenyl alpha naphthylamine                            | 0.5                          | 0.5              | 0.375            | 0.375   |
| Mineral lubricating oil                               |                              |                  |                  |         |
| 55 SUS at 210°F                                       | 81.5                         | 71.5             | 53.625           | 61.125  |
| 70 SUS at 210°F                                       |                              |                  | 25.0             | 25.00   |
| Properties:                                           |                              |                  |                  |         |
| Appearance                                            | Smooth, uniform, short fiber |                  |                  |         |
| Dropping Point (°F.)                                  | 500+                         | 500+             | 500+             | 500+    |
| Penetrations (77°F. mm./10)                           |                              |                  |                  |         |
| Unworked                                              | 282                          | 245              | 310              | 315     |
| Worked 60 strokes                                     | 292                          | 285              | 315              | 330     |
| Worked 100,000 strokes (125°F.)                       | 340                          | 245              |                  |         |
| Cooled to 77°F.—60 additional strokes                 | 339                          | 325              |                  |         |
| Wheel Bearing Test (220°F. 6 hours 660 R. P. M.)      | Pass                         | Pass             |                  |         |
| Timken Test (lb. load)                                | 30 Fall                      | 60 (narrow scar) | 40 (narrow scar) | 30 Fall |
| Norma Hoffman Oxidation Test (hrs. to 5 p. s. 1 drop) | 365                          | 385              |                  |         |
| Lubrication Life (hrs.) (250°F.—10,000 R. P. M.)      | 2,100                        | 2,200            | NIL              |         |
| Water Solubility                                      |                              |                  |                  |         |

It will be noted that Grease B has an outstanding load carrying ability in addition to other desirable grease characteristics. Furthermore, when Grease B is diluted or blended with additional lubricating oil it retains an adequate load carrying ability although the grease is softer in structure. When Greases B and C, the preferred lubricating grease compositions of the invention, are compared to Greases A and D, the new and unexpected results of this invention are clearly indicated.

The invention is not limited to the specific conditions and materials of the foregoing example. These conditions and materials may be varied within the limits indicated in the general portions of the specification. The grease compositions prepared in accordance with the invention may also contain various conventional additives such as oxidation inhibitors, metal deactivators, corrosion inhibitors, extreme pressure agents, etc. as will be understood by those skilled in the art.

What is claimed is:

1. A soap-salt complex comprising a metal salt of a low molecular weight monocarboxylic acid having in the range of 1 to 3 carbon atoms per molecule, a metal salt of an ethylene diamine tetra aliphatic carboxylic acid, the carboxylic groups thereof having in the range of 1 to 4 carbon atoms, and a metal soap of a high molecular weight carboxylic acid having in the range of 12 to 30 carbon atoms per molecule, said complex being formed at a complex-forming temperature in the range of 400°-550° F. and containing in the range of 5 to 20 parts by weight of said low molecular weight monocarboxylic acid, 1 to 5 parts by weight of said ethylene diamine tetra aliphatic carboxylic acid, and 3 to 15 parts by weight of said high molecular weight carboxylic acid, and the metal constituent of said metal salts and soap being an alkaline earth metal.

2. The complex of claim 1 wherein said ethylene diamine tetra aliphatic carboxylic acid is ethylene diamine tetra acetic acid, and said low molecular weight monocarboxylic acid is acetic acid.

3. A lubricating grease composition comprising a mineral lubricating oil thickened to a grease consistency within the range of 3 to 50 wt. percent of a soap-salt complex consisting of a metal salt of in the range of 5 to 20 wt. percent of a low molecular weight monocarboxylic acid having in the range of 1 to 3 carbon atoms per molecule, a metal salt of in the range of 1 to 5 wt. percent of an ethylene diamine tetra aliphatic carboxylic acid, the carboxylic acid groups thereof having in the range of 1 to 4 carbon atoms, and a metal soap of in the range of 3

to 15 wt. percent of a high molecular weight carboxylic acid having in the range of 12 to 30 carbon atoms per molecule, the weight percentages being based on the total grease composition, the metal constituent of said metal salts and soap being an alkaline earth metal and said complex being formed at a complex-forming temperature in the range of 400° to 550° F.

4. The grease composition of claim 3 wherein said low molecular weight monocarboxylic acid is acetic acid.

5. The lubricating grease composition of claim 3 wherein said alkaline earth metal is calcium.

6. The process of preparing a lubricating grease composition which comprises dispersing in a mineral lubricating oil in the range of 3 to 15 wt. percent of a high molecular weight carboxylic acid having in the range of 12 to 30 carbon atoms per molecule, in the range of 1 to 5 wt. percent of an ethylene diamine tetra aliphatic carboxylic acid, the carboxylic acid groups thereof having in the range of 1 to 4 carbon atoms, and in the range of 5 to 15 wt. percent of an alkaline earth metal base, heating the resulting dispersion to a temperature in the range of 80° to 150° F., then adding in the range of 5 to 20 wt. percent of a low molecular weight monocarboxylic acid having in the range of 1 to 3 carbon atoms per molecule, continuing heating the mixture to a complex-forming temperature in the range of 400° to 550° F., and then cooling the mixture to obtain said lubricating grease composition.

7. The process of claim 6 wherein said ethylene diamine tetra aliphatic carboxylic acid is ethylene diamine tetra acetic acid, wherein said low molecular weight monocarboxylic acid is acetic acid, and wherein said alkaline earth metal is calcium.

60 References Cited in the file of this patent

UNITED STATES PATENTS

|              |                   |               |
|--------------|-------------------|---------------|
| 2,197,263    | Carmichael et al. | Apr. 16, 1940 |
| 2,240,957    | Munz              | May 6, 1941   |
| 65 2,412,944 | Bersworth         | Dec. 24, 1946 |
| 2,417,428    | McLennan          | Mar. 18, 1947 |
| 2,564,561    | Carmichael et al. | Aug. 14, 1951 |
| 2,583,607    | Sirianni et al.   | Jan. 29, 1952 |
| 2,628,195    | Allison et al.    | Feb. 10, 1953 |

70 OTHER REFERENCES

The Institute Spokesman, vol. 14, No. 12, March 1951 (Amott and McLennan Article), pages 7-23.  
Boner: "Lubricating Greases," chapter 16, pages 615-73 675, Reinhold Pub. Corp., New York, N. Y.